

# UNITED STATES PATENT OFFICE.

FREDERICK C. OVERBURY, OF HILLSDALE, NEW JERSEY, ASSIGNOR, BY MESNE  
ASSIGNMENTS, TO THE FLINTKOTE COMPANY, OF BOSTON, MASSACHUSETTS,  
A CORPORATION OF MASSACHUSETTS.

## PREPARED MINERAL-SURFACED ROOFING.

1,314,753.

Specification of Letters Patent.

Patented Sept. 2, 1919.

No Drawing.

Application filed October 16, 1915. Serial No. 56,289.

*To all whom it may concern:*

Be it known that I, FREDERICK C. OVERBURY, a citizen of the United States, residing at Hillsdale, in the county of Bergen and 5 State of New Jersey, have invented new and useful Improvements in Prepared Mineral-Surfaced Roofing, of which the following is a specification.

This invention has relation to prepared 10 roofing fabrics of that type in which the facing or coating consists of a relatively thick layer of crushed slate or analogous mineral material more or less embedded in a layer of asphalt or pitch. In such fabrics, 15 the foundation consists of fibrous material impregnated or saturated with a bituminous or hydrocarbon compound having a relatively low melting point while the latter is soft and fluid, and upon this foundation so 20 treated is applied a layer of molten pitch or asphalt, or other bituminous compound, in which the surface coating of crushed mineral is embedded while the pitch or asphalt is in a plastic adhesive condition. Such 25 roofing fabrics are pleasing and attractive, since the slate or other crushed mineral may be obtained in different colors or tints, and many different color effects can be secured.

Several difficulties have arisen in the marketing of such roofing fabrics, one of which 30 is that, after the goods are manufactured and are prepared for shipment, either in rolls when in sheet form, or in flat packages when in strip or shingle form, there are certain 35 oils or oily matters which sometimes find their way from the bituminous coating into the layer of slate or other mineral and discolor it. The result is that in different batches held in stock, although the mineral 40 surfaces may be formed from the same raw material, they differ in tint or shade, and, when laid on the same roof, produce an un- 45 pleasing and unsatisfying result. The object of this invention is to overcome this difficulty. I find that I can accomplish the ob- 50 ject by spraying or treating the surface coating of slate with some non-oily compound which is not a solvent of asphalt or pitch and which will prevent the oil or oily com- 55 pound in the pitch or asphalt from reaching the surface of the mineral. For this purpose, I may employ, for example, sodium silicate, or a solution of soap bark or even

a thin glue solution, and many other compounds which are more or less transparent 55 and which will readily suggest themselves to one skilled in the art. The sprayed compound should quickly dry on the crushed mineral surface. In practice, after the sheet of roofing has been surfaced in the usual 60 manner with the crushed mineral, I feed it under the spray, which should be finely divided so as not to unduly wet the sheet. The sprayed compound settles and collects any mineral dust which may be on the sheet. 65 The sheet is then rolled, or cut and packaged. Instead of applying the compound as a spray, it may be applied in other ways.

It is not my object to fill the pores of the rough mineral facing of the roofing material 70 to produce a smooth surface, or ultimately to change the roughness of the coating. Consequently I employ only those substances which in solution or suspension can be applied to the roofing material without changing 75 its character and which are approximately transparent or of such nature as not to hide the general color and appearance of the mineral facing. By the use of a substance as herein suggested, I prevent discoloration of the mineral facing by the oily components of the waterproofing material, and also impart a uniform appearance thereto.

Having thus explained the nature of my 85 invention and a way of practising the same, although without attempting to set forth all of the ways in which it may be practised, what I claim is:

1. The herein described method of making 90 mineral surfaced waterproof roofing fabric, which includes treating the mineral surface with a compound substantially transparent in thin layers to prevent subsequent change in the color or tint thereof due to oily mat- 95 ters contained in such fabric, without changing the rough character and appearance of such mineral surface.

2. The herein described method of making 100 mineral surfaced waterproof roofing fabric, which includes coating said fabric with a bituminous compound, covering said coating with a layer of crushed slate or equivalent mineral, and spraying said layer with a liquid compound substantially transparent 105 in thin layers to prevent subsequent change

of color or tint due to the action thereon of oily matter contained in said bituminous compound, without changing the rough character and appearance of such mineral surface.

- 5 3. The herein described method of making mineral surfaced waterproof roofing fabric, which includes coating said fabric with a bituminous compound, covering said coating 10 with a layer of crushed slate or equivalent mineral and spraying said layer with a liquid non-oily compound which is a non-solvent of the bituminous compound to protect said mineral from the oily matters contained in said bituminous compound, without 15

changing the rough character and appearance of such mineral surface.

4. A weatherproof roofing fabric having a bituminous coating and a layer of crushed slate or equivalent mineral embedded therein, and a thin transparent coating on said crushed mineral to protect it against subsequent change in color due to oily substances contained in said bituminous coating, without changing the rough character 20 and appearance of such mineral surface.

In testimony whereof I have affixed my signature.

FREDERICK C. OVERBURY.